

Oct. 24, 1950

P. H. CARNELL

2,526,931

COLOR AND VISCOSITY OF LUBRICATING OILS

Filed Dec. 15, 1947



INVENTOR.  
P. H. CARNELL

BY *Hudson and Young*

ATTORNEYS

## UNITED STATES PATENT OFFICE

2,526,931

## COLOR AND VISCOSITY OF LUBRICATING OILS

Paul H. Carnell, Alma, Mich., assignor to Phillips Petroleum Company, a corporation of Delaware

Application December 15, 1947, Serial No. 791,802

4 Claims. (Cl. 196—39)

1

This invention relates to the treatment of lubricating oils to improve their properties. In one of its more specific aspects it relates to a treatment of a lubricating oil which improves its color and viscosity or viscosity index.

I have discovered that treatment of a lubricating oil with hydrofluoric acid and molybdenum sulfide, at elevated temperature and pressure, will improve the ASTM color of the oil, and also the viscosity index. In one embodiment of this invention, hydrogen is added to the hydrofluoric acid, molybdenum sulfide, and oil. One effect of the inclusion of hydrogen is to aid in prolonging the life of the hydrofluoric acid.

Lubricating oil, as referred to herein, includes all such products and their base stocks which have a viscosity within the range of about 75 SUS (Saybolt Universal seconds) at 100° F. to about 150 SUS at 210° F., and as are usually understood to be covered by this term by those skilled in the art. It includes, particularly, lubricating oil stocks, such as, paraffin-base stock, naphthene-base stock, synthetic-base stock, and mixed-base stock, which are refined for use as engine lubricants. By blending various " neutrals" and "bright stocks," engine lubricating oils of varying viscosities and viscosity indices are produced.

The hydrofluoric acid, hydrogen, and molybdenum sulfides, used in the practice of this invention, may be of the quality of the commercial products. The hydrofluoric acid, referred to as substantially anhydrous hydrofluoric acid, is commercial hydrofluoric acid, and may contain small amounts of sulfur dioxide, water, and other impurities. The words "molybdenum sulfide," as referred to in this invention, mean any sulfide of molybdenum.

An object of the present invention is to provide a novel and improved method for improving lubricating oils. Another object is to provide a method for improving natural lubricating oils. Another object is to provide a method for improving mixed-base lubricating oils. Another object is to provide a method for improving synthetic-base lubricating oils. Another object is to provide a method for improving the color and viscosity index of natural or synthetic lubricating oils. Another object is to provide a method for improving the color of a lubricating oil. Other objects and advantages of this invention will become apparent from the accompanying disclosure and discussion.

Broadly speaking, my invention comprises a process of improving lubricating oil by contact-

2

ing the lubricating oil with substantially anhydrous hydrofluoric acid and at least one molybdenum sulfide, such as, molybdenum disulfide, at elevated temperature and pressure.

Treatment of lubricating oil with hydrofluoric acid in combination with various other materials, such as, metallic oxide, phenols, alcohols, sulfur dioxide, etc., is well known. At temperatures where such treatment satisfactorily improves the viscosity index, the color of the lubricating oil is often impaired. Improvement in color generally is obtained only when the oil is treated at a temperature of 30° C. or lower, and, in general, at this temperature very little improvement in viscosity index is obtained. My invention incorporates improvement in color as well as in viscosity index, at elevated temperatures, by treating a lubricating oil with hydrofluoric acid and at least one molybdenum sulfide. Olefins, aromatics, unsaturated resins, gum-forming bodies, and other undesirable components are removed by the hydrofluoric acid, improving the general properties of the oil. The color is improved by the molybdenum sulfide. The advantage of this process is the improvement of color in the same step with improvement of viscosity index.

In general, lubricating oil, substantially anhydrous hydrofluoric acid, and one or more molybdenum sulfides are introduced to a contact chamber for a time within the range of about 40 to about 180 minutes, at an elevated temperature within the range of about 100 to about 300° C., and pressure within the range of about 500 to about 1500 pounds per square inch. The proportion of lubricating oil to hydrofluoric acid of about 1:20 to about 20:1 is recommended, however, only enough hydrofluoric acid need be present to make a definite acid phase. The amount of molybdenum sulfide recommended is in the range of about 5 to about 20 weight per cent of the oil being treated; however, more may be added, if desired, but little is gained by amounts larger than 20 weight per cent, and too much will clog the apparatus. After contacting the hydrofluoric acid-oil-molybdenum sulfide mixture in the reactor it is transferred to an agitator where a light paraffin, such as, iso- or normal butane, or iso- or normal pentane, is added to aid in breaking the hydrofluoric acid-oil emulsion, and which may also react to some extent with the treated mixture. From the agitator the mixture is passed to a settler unit where it is separated into an oil-light hydrocarbon layer and a hydrofluoric acid-molybdenum sulfide-acid solution oil layer. The improved lubricating oil

is then separated from the oil-light hydrocarbon layer and recovered.

This process may be carried out either in a batchwise manner or continuously, the latter being preferred for commercial operation. A better understanding of my invention may be had by referring to the accompanying schematic flow diagram of a preferred embodiment of the invention.

Referring to Figure 1 of the attached diagram, hydrofluoric acid, lubricating oil, and molybdenum sulfide are introduced to reactor 13 through lines 10, 11, and 12, respectively. This mixture is agitated at an elevated temperature between about 100 to about 300° C. and pressure between about 500 to about 1500 pounds per square inch. The treated mixture from reactor 13 is passed through line 14 to agitator 16 where it is agitated with a light paraffin introduced through line 17, such as, isopentane, to break the hydrofluoric acid-oil emulsion. From agitator 16 the hydrofluoric acid-oil-molybdenum sulfide-light paraffin mixture is passed through line 18 to settler 19. In settler 19 the mixture is separated into two layers; an upper layer of treated oil and light hydrocarbons, and a lower layer of hydrofluoric acid, molybdenum sulfide, and acid soluble materials. The lower layer is passed through line 21 to fractionator 22 where relatively pure hydrofluoric acid is separated and recycled to reactor 13 through lines 23 and 10, respectively. The acid soluble oil and molybdenum sulfide are withdrawn from the kettle of fractionator 22 through line 24 to a molybdenum sulfide recovery unit 26. The recovered molybdenum sulfide is recycled to reactor 13 through lines 27, 28, and 12. The upper layer from settler 19 is passed through line 29 to fractionator 31 where the light paraffin used to break the hydrofluoric acid-oil emulsion is separated for recycle to agitator 16 through lines 32, 33, and 17. Other relatively light hydrocarbons from fractionator 31, formed in the high temperature hydrofluoric acid treatment, may be recovered as by-products of the process through line 35, or recycled to reactor 13 through lines 36 and 11. The improved lubricating oil is withdrawn from the kettle of fractionator 31 through line 34 as a product of the process, and may be caustic-washed and/or filtered, if desired. Any small amount of hydrogen sulfide formed in this process by the reaction of a molybdenum sulfide with hydrofluoric acid may be suitably recovered as a by-product of the process.

Any suitable equipment may be employed in the performance of the present invention, and particularly equipment which is resistant to the corrosive action of hydrofluoric acid. Conventional contacting equipment, similar to contactors which are commonly used for conducting the alkylation of aliphatic isoparaffins and olefins, may be used to provide suitable contact between the reactants. Any other means of maintaining an intimate contact of the lubricating oil and acid-sulfide phase may be employed. The equipment should be provided with means for maintaining the desired temperatures and pressures in the various zones.

To further illustrate some of the many aspects of this invention the following specific example is given.

#### Example I

A 4½ liter steel bomb was charged with hydrofluoric acid and a mixed-base lubricating oil. In particular runs, molybdenum disulfide and/or hydrogen were also charged to the bomb. The charged reaction bomb was fitted with a suitable

pressure gauge and heating equipment and then clamped on a platform rocker. The bomb was heated and agitated for a given contact time, and then allowed to cool to room temperature. After cooling, the bomb was charged with 1 liter of isopentane. The resulting mixture was agitated one hour, and then removed from the rocker and allowed to stand in a vertical position for 1 hour. The acid layer was withdrawn, and the hydrocarbon layer was washed with caustic, filtered, and topped to the initial boiling point of the untreated oil at reduced pressure, to remove light ends. The following data were obtained.

| Run                               | Un-treated Oil | 1     | 2     | 3     | 4     |
|-----------------------------------|----------------|-------|-------|-------|-------|
| HF, grams                         |                | 581   | 595   | 994   | 999   |
| Oil, grams                        |                | 869   | 865   | 876   | 873   |
| Molybdenum disulfide, grams       |                |       |       | 50    | 50    |
| Hydrogen, p. s. i.                |                |       | 200   |       | 300   |
| Contact time, minutes             |                | 120   | 120   | 120   | 120   |
| Contact temperature, °C. (max.)   |                | 172   | 174   | 169   | 158   |
| Contact pressure, p. s. i. (max.) |                | 740   | 960   | 650   | 980   |
| Physical Constants:               |                |       |       |       |       |
| Viscosity, 100 F, SUS             | 388.3          | 335.9 | 342.0 | 348.8 | 343.3 |
| Viscosity, 210 F, SUS             | 55.52          | 54.93 | 54.59 | 55.20 | 55.00 |
| Viscosity index (Dean & Davis)    |                | 85    | 101   | 96    | 98    |
| API gravity                       | 28.4           | 30.5  | 30.1  | 31.0  | 30.4  |
| ASTM color                        | 3½             | 4     | 4     | 3     | 3     |

The data from runs 1 and 2 show that treatment of a mixed-base lubricating oil with hydrofluoric acid at elevated temperatures and pressures, in the presence and in the absence of hydrogen, produces oils of improved viscosity index, but impaired color.

The data from runs 3 and 4 show that treatment of the same mixed-base lubricating oil with hydrofluoric acid and molybdenum disulfide, at elevated temperatures and pressures, and in the presence and in the absence of hydrogen, produces oils of improved color and also viscosity index, as described in this invention.

In runs 2 and 4 hydrogen was introduced to increase the pressure within the bomb, and to prolong the life of the hydrofluoric acid.

Although the process has been described and exemplified in terms of its preferred modifications, it is understood that various changes may be made without departing from the spirit of the process as disclosed and expressed in the claims.

I claim:

1. The process of manufacturing a lubricating oil of improved color and viscosity index, which comprises treating a lubricating oil with a mixture of substantially anhydrous hydrofluoric acid and at least one molybdenum sulfide, the ratio of hydrofluoric acid to oil being in the range of about 1:20 to about 20:1, and the quantity of molybdenum sulfide being in the range of about 5 to about 20 weight per cent of the oil being treated, said treatment of lubricating oil taking in the range of about 100 to about 300° C. at a pressure sufficient to maintain the oil and hydrofluoric acid in liquid phase which is in the range of about 500 to about 1500 pounds per square inch, for a period of time within the range of about 40 to about 180 minutes, cooling said mixture of oil, hydrofluoric acid, and molybdenum sulfide, introducing a light-paraffin to break the acid-oil emulsion, and recovering an improved lubricating oil as a product of the process.

2. The process according to claim 1, in which the molybdenum sulfide used is molybdenum di-

3. A process for manufacturing a lubricating oil of improved color and viscosity index, which comprises treating a lubricating oil with a mixture of substantially anhydrous hydrofluoric acid and a molybdenum disulfide, the ratio of hydrofluoric acid to oil being in the range of 1:20 to 20:1, and a quantity of molybdenum disulfide being in the range of 5 to 20 weight per cent of the oil being treated, treating said oil at a temperature in the range of 100 to 300° C., a pressure in the range of 500 to 1500 pounds per square inch and for a period of time within the range of 40 to 180 minutes, accomplishing said treatment in a hydrogen atmosphere, cooling the mixture of oil, hydrofluoric acid and molybdenum disulfide and introducing thereto a light paraffin to break the acid-oil emulsion, and recovering an improved lubricating oil as a product of the process.

4. In a process according to claim 3, the use of a hydrogen atmosphere under a partial pressure of 200 to 300 pounds per square inch.

PAUL H. CARNELL.

5 REFERENCES CITED

The following references are of record in the file of this patent:

10 UNITED STATES PATENTS

| Number    | Name     | Date          |
|-----------|----------|---------------|
| 2,366,743 | Matuszak | June 9, 1945  |
| 2,378,762 | Frey     | June 19, 1945 |

15 FOREIGN PATENTS

| Number  | Country       | Date         |
|---------|---------------|--------------|
| 292,932 | Great Britain | May 23, 1929 |